

## UNITED STATES PATENT OFFICE

WILLIAM A. MUDGE, OF HUNTINGTON, WEST VIRGINIA, ASSIGNOR, BY MESNE ASSIGNMENTS, TO THE INTERNATIONAL NICKEL COMPANY, INC., OF NEW YORK, N. Y., A CORPORATION OF DELAWARE

HEAT-TREATED NICKEL-COPPER-ALUMINUM ALLOY AND METHOD OF HEAT TREATING THE SAME

No Drawing.

Application filed June 10, 1924. Serial No. 719,088.

My invention relates to the treatment of alloys containing as their main ingredients nickel, copper and aluminum, and it may be applied to any ternary alloy containing these three metals as its major ingredients, wherein the aluminum content is preferably not over 20%.

In the manufacture of such alloys, a wide variation in the physical properties of the product, even when of constant composition, has been observed, and no reason could be assigned for such variations, inasmuch as the alloy was supposed to be a true solid solution.

I have discovered that this alloy is not a true solid solution and that the physical properties of a constant composition thereof may be changed to a considerable degree by heat treatment. I believe this to be due to the formation, during heating above 500-2000° F., of a compound between two of the constituents, namely, copper and aluminum. I have found that the amount of this compound, even in a constant composition of alloy, varies in accordance with the heat treatment, and, therefore, I believe that it gives the variation in physical characteristics. The amount of this compound will also vary with different compositions, even under the same heat treatment.

In a long series of experiments on heat treatment of this material, I have made the following discoveries:

If the material has been quenched from a temperature above 1500° F., it will be dead soft. If such dead soft material is heated, I have found the following facts:

- (a) Up to about 600° F., there will be practically no change in the physical properties.
- (b) Between 600° F. and 1000° F., a gradual increase in desirable physical properties and hardness will result; and
- (c) At a range from 1000° F. to 1200° F., the maximum desired properties will be developed.

By "physical properties" in the above statement, I mean that the proportional limit, yield point, and ultimate strength and hardness will be increased, while the elongation and reduction of area will be decreased.

The above statements apply regardless of

the rate of cooling, but slow cooling from any of the temperatures above mentioned will, in general, give better physical properties than when the material is rapidly cooled from these same temperatures, as for example, by quenching in oil or water or in any other suitable quenching medium.

If the material is heated to a temperature above 1200° F., there will be a decrease in these physical properties, and this decrease will be proportional to the increase in temperature from 1200° F. up to below 1800° F.

Also the rate of cooling will affect the desired physical properties in this case. When rapidly cooled or quenched, the desired properties will be slightly lower than when slowly cooled from the same temperatures.

Also, there is a time effect in the heating, since extending the time of heating tends to increase the desired physical properties. For example, using dead soft material and one hour's heating at the best temperature of about 1100° F., would give semi-hard material, whether cooled slowly or rapidly; whereas, if this heating at this same temperature on the same material was continued for eight or more hours, a hard material will be produced having physical properties considerably in excess of those produced in one hour's heat treatment; and this again, whether the cooling is rapid or slow.

Continued heating at the maximum temperature of about 1100° F. for more than eight hours will slightly, but definitely, increase the physical properties regardless of the rate of cooling.

As specific illustrations of these treatments, I will recite the following examples, the material treated being composed of approximately 66% nickel, 26% copper, 4% aluminum, together with 4% iron and manganese and .19% of carbon as minor constituents.

*1st example.*—Original material whose proportional limit was 92,000 lbs. psi. was quenched from 1500° F., which reduced its value to 25,000 lbs. psi. Heating at 1100° F. raised the proportional limit from its original 25,000 lbs. psi. up to 70,000 lbs. psi. during the first hour. The proportional limit was raised to 94,000 lbs. psi. at the end of the

seventh hour and to 97,000 lbs. psi. at the end of the forty-eighth hour. In this case, all the heating was carried out at 1100° F. and followed by slow cooling in air, but the same results might have been accomplished by rapid cooling following the same heat treatment.

It will be noted from this example that starting with an original material of high physical properties, the heat treatment reduces these physical properties to a minimum and then raises them beyond the original values, all by heat treatment and without mechanical working.

Similar results to those above recited have been obtained with a composition containing 15 45% of nickel, 55% of copper, 4% of aluminum, together with 1.5% of iron and manganese and .06% carbon as minor constituents.

20 *2nd example.*—When this alloy has been hardened and the desired physical properties developed to a high value by the heat treatment, such as before described, it may be heated in the following ways without affecting 25 its properties:

(a) To any temperature not to exceed 1300° F. with slow cooling.

(b) To any temperature not exceeding 1200° F. with quenching or quick cooling.

30 This discovery is important, especially in using the material in locations where it is subjected to variations in temperature conditions; as, for example, when used for steam turbine blades. The maximum temperature

35 in turbine work is lower than the above points, and hence, the material will retain its desired physical properties under these conditions, even under wide variations of temperature.

40 In other words, intermittent service at or below these temperatures does not materially change the characteristics of the material, if tested when cooled down.

If the material is heated above these temperatures, a decrease in the desired physical 45 properties will result, without regard to the rate of cooling; but if the material is slowly cooled after such heating, it will have higher properties than if quenched after heating to above such temperatures.

50 *3rd example.*—If this hardened material is heated to a point between 1200 and 1500° F., a semi-hard material will be produced, regardless of the rate of cooling; although the 55 slowly cooled material in this case will be slightly harder than the quenched or rapidly cooled material. If this hardened material is heated to above 1500° F., and quenched or rapidly cooled, it will produce dead soft material; while slowly cooling it from a temperature of 1500° F. or above, will produce a semi-hard material.

The above examples recite the major discoveries which I have made in my heat treatment research on such alloys. I will now de-

scribe certain other features which I have found in this research.

Either the dead soft or semi-hard alloy, when these properties have been imparted by the proper heat treatments, can be machined or fabricated with about the same ease as a similar nickel-copper alloy containing no aluminum.

If the material is hardened and has the desired physical properties to a high degree, it is machined with considerable difficulty. Therefore, anyone machining or fabricating this material while relatively cold and without material heating, to obtain a certain article or device, would probably desire it in soft or semi-hard condition for such treatment; and thereafter the desired physical properties can be imparted by heating at from 1000° F. to 1200° F., the properties increasing with the length of heating, as above described, and being preferably followed by a slow cooling to bring these properties to their highest values.

Where the material is worked in hot condition for sale in merchant shapes, the best 90 practice would probably be to roll or forge it at a temperature between 1800° F. and about 2150° F., with ordinary slow cooling in the air. This will give a semi-hard product, without any further treatment, and if the customer desired a dead soft material, the material as rolled or otherwise hot worked should be quenched or quickly cooled from a temperature above 1500° F. to give a soft material.

If, on the other hand, a customer desired a very hard alloy, possessing the desired physical properties to a high degree, the best practice would be to allow the material to cool slowly after hot working at the above temperatures, and then to heat the material at from 1000° to 1200° F. for several hours and allow it to cool slowly in the air. As above pointed out, the longer this heating extends within certain limits, the more of the compound will be formed and the greater the physical characteristics.

110 My belief is that the hardness and other desired physical properties are due to the gradual formation of the copper-aluminum compound during the heating at a temperature between 1000° F. and 1200° F.

I have also found that where the desired properties are imparted, either to a high degree or to a medium degree, these properties are slightly improved by aging the material. Thus, where the material has been quenched from above 1500° F. to produce dead soft material, the proportional limit being reduced from 92,000 lbs. psi. to 25,000 lbs. psi., this material was heated at about 1100° F. for two hours, and some samples quenched and others slowly cooled.

115 In both cases one sample was tested about five minutes after cooling and another about 130

19 hours after cooling. The aged samples from both the quenching and the slow cooling were found to be improved in proportional limit, by from 5 to 15%.

5 The advantages of my invention will be apparent to those skilled in the art, since the heat-treating of this alloy, in accordance with the above discoveries, enables its properties to be varied as desired, and definite and uniform results obtained in the desired physical properties of the alloy and in accordance with the characteristics desired.

10 The relative proportions of the alloy may be varied, the percentages of other ingredients may be changed, and other variations may be made, without departing from my invention.

I claim:

1. In the treatment of nickel-copper-aluminum alloys containing less than 20% of aluminum and at least 15% of nickel, the steps consisting of heating the material to above 600° F. and allowing it to cool.

2. In the treatment of nickel-copper-aluminum alloy containing less than 20% of aluminum and at least 15% of nickel, the steps consisting of heating the material and subjecting it to a regulated cooling action, the heating and cooling being sufficient to change the physical properties.

3. In the treatment of nickel-copper-aluminum alloy containing less than 20% of aluminum and at least 15% of nickel, the steps consisting of heating the material to above 600° F. and subjecting it to a regulated cooling action.

4. In the treatment of nickel-copper-aluminum alloy containing less than 20% of aluminum and at least 15% of nickel, the steps consisting of heating the material to between 600° F. and 1000° F. and subjecting it to regulated cooling.

5. In the treatment of nickel-copper-aluminum alloy containing at least 15% of nickel and less than 20% aluminum, the steps consisting of subjecting the material to a temperature between 1000° F. and 1200° F. and subjecting it to a regulated cooling.

6. In the treatment of nickel-copper-aluminum alloy containing less than 20% of aluminum and at least 15% of nickel, the steps consisting of heating the material to between 1000° F. and 1200° F. and allowing it to cool.

7. In the treatment of nickel-copper-aluminum alloy containing less than 20% of aluminum and at least 15% of nickel, the steps consisting of heating the material to between 1200° F. and 1500° F. and allowing it to cool.

8. In the treatment of nickel-copper-aluminum alloy containing less than 20% of aluminum and at least 15% of nickel, the steps consisting of rapidly cooling a hard

alloy containing nickel, copper and aluminum to soften it, and then heating same at temperature between 600° F. and 1200° F. and allowing it to cool.

9. In the treatment of nickel-copper-aluminum alloy containing less than 20% of aluminum and at least 15% of nickel, the steps consisting of rapidly cooling a hard alloy containing nickel, copper and aluminum to soften it, and then heating same at temperature between 600° F. and 1200° F. and slowly cooling same.

10. As a new article of manufacture, an alloy whose major constituents are nickel, copper and aluminum, one of the other metals being present to a greater percentage than the aluminum, the aluminum being less than 20% and the nickel being at least 15%, said alloy having a physical structure such as is produced by heat treating an alloy of this composition to above 600° F. and allowing it to cool.

11. As a new article of manufacture, an alloy whose major constituents are nickel, copper and aluminum, one of the other metals being present to a greater percentage than the aluminum, the aluminum being less than 20% and the nickel being at least 15%, said alloy having a physical structure such as is produced by heat treating an alloy of this composition to between 1000 and 1200° F. and allowing it to cool.

12. As a new article of manufacture, an alloy whose major constituents are nickel, copper and aluminum, one of the other metals being present to a greater percentage than the aluminum, the aluminum being less than 20% and the nickel being at least 15%, said alloy having a physical structure such as is produced by heat treating an alloy of this composition to between 1200° and 1500° F. and allowing it to cool.

In testimony whereof I have hereunto set my hand.

WILLIAM A. MUDGE. 110

115

120

125

130